

[54] STEEL ALLOY

[75] Inventors: Thomas Watmough, Dolton; Robert P. O'Shea, Lombard, both of Ill.

[73] Assignee: The United States of America as represented by the Secretary of the Air Force, Washington, D.C.

[22] Filed: Aug. 14, 1972

[21] Appl. No.: 280,281

[52] U.S. Cl. .... 75/126 D, 75/126 E, 102/67

[51] Int. Cl. .... C22c 39/26, F42b 13/48

[58] Field of Search ..... 75/126 R, 126 D, 75/126 E, 123 N, 123 L; 102/67

## [56] References Cited

## UNITED STATES PATENTS

|           |         |                    |            |
|-----------|---------|--------------------|------------|
| 3,664,830 | 5/1972  | Kambayashi.....    | 75/126 D X |
| 3,600,161 | 8/1971  | Inouye et al. .... | 75/126 D X |
| 3,251,682 | 5/1966  | Wada.....          | 75/126 D   |
| 3,044,872 | 7/1962  | Hayes .....        | 75/126 D   |
| 2,968,549 | 1/1961  | Brady et al. ....  | 75/126 D   |
| 2,858,206 | 10/1958 | Boyce et al. ....  | 75/126 D   |

|           |         |                    |          |
|-----------|---------|--------------------|----------|
| 2,737,455 | 3/1956  | Kirkby et al. .... | 75/126 D |
| 2,683,086 | 7/1954  | Clark .....        | 75/126 D |
| 2,040,189 | 5/1936  | Strauss.....       | 75/126 D |
| 3,547,032 | 12/1970 | Horvath .....      | 102/67   |

## FOREIGN PATENTS OR APPLICATIONS

1,200,423 7/1970 Great Britain ..... 75/126 D

## OTHER PUBLICATIONS

Roberts et al., Tool Steels, 3rd Ed. American Society for Metals, Metals Park, Ohio, 1962, pp. 227, 718.

Primary Examiner—Carl D. Quarforth

Assistant Examiner—R. E. Schafer

Attorney—Harry A. Herbert, Jr. et al.

## [57] ABSTRACT

A low alloy steel having titanium as an essential alloying ingredient. The titanium addition provides the means for controlling and manipulating the fragment mass distribution characteristics emanating from the detonation of an explosive warhead fabricated from the titanium containing steel alloy.

4 Claims, 2 Drawing Figures

PATENTED JAN 15 1974

3,785,804



FIG. 1



FIG. 2

## STEEL ALLOY

## BACKGROUND OF THE INVENTION

This invention relates to a low alloy steel having titanium as an alloying ingredient. In a more particular manner, this invention is concerned with the use of titanium as a means for controlling the fragmentation characteristics of low alloy tempered martensitic steels used in warheads.

The distribution patterns and fragmentation characteristics of steel fragments produced by a detonating warhead is a problem of great concern to those responsible for the fabrication and design of antipersonnel and antivehicle weapons. The effectiveness of grenades, artillery and mortar shells, aerial bombs and other explosive warheads depends to a great extent upon the fragmentation characteristics of the materials used to fabricate such weapons. In an attempt to improve their fragmentation effects, it has been found that the incorporation of titanium as an essential alloying ingredient in low alloy tempered martensitic steels provides a component that is extremely useful as a structural material for warheads. It provides a means for controlling the fragment mass distribution effect in such a manner that the weapons can be employed against both light and heavy targets.

## SUMMARY OF THE INVENTION

In accordance with the broad concept of this invention, it has been found that the inclusion of titanium in low alloy steels having a tempered martensitic structure provides a means for controlling the fragment mass distribution characteristics of those alloys when they are employed in the manufacture of explosive warheads. The titanium is a ferrite strengthener and a carbide stabilizer and as such can provide an embrittled structure that controls fragmentation.

Still another object of this invention is to provide a structural material that possesses the type of fragment mass distribution characteristics that make it useful in the manufacture of explosive warheads for use against both light and heavy military targets.

The above and still further objects and advantages of the present invention will become readily apparent upon consideration of the following detailed description thereof when taken in conjunction with the following drawings.

## DESCRIPTION OF THE DRAWINGS

In the drawings:

FIG. 1 and 2 are graphical representations showing the effects of titanium content on the fragment mass distribution characteristics of the alloys of this invention.

## DESCRIPTION OF THE PREFERRED EMBODIMENTS

The fragmentation alloys of this invention are low alloy steels of medium carbon content that possess a tempered martensitic structure. The addition of titanium, as an essential alloying ingredient, provides the means for producing an embrittled ferrite structure that controls the fragmentation characteristics of the martensitic steel alloys of this invention.

The titanium is incorporated in the alloy in specified amounts in accordance with conventional alloying techniques. The titanium is a ferrite strengthener and carbide stabilizer and produces the embrittled structure which controls the fragmentation characteristics of the alloy. A medium carbon low alloy steel of varying composition, with three levels of titanium, was selected to verify if titanium additions could control the fragmentation effects in both forged and cast steels.

The compositions of the steel alloys of this invention are given in Table I.

TABLE I

## COMPOSITION OF TITANIUM-BEARING STEELS

| Example | Structure | Analysis, weight percent |      |      |      |      |      |     |
|---------|-----------|--------------------------|------|------|------|------|------|-----|
|         |           | C                        | Mn   | Si   | Cr   | V    | Ti   | Fe  |
| 1       | Forged    | 0.51                     | 1.30 | 0.50 | 1.16 | 0.21 | 0.28 | bal |
| 2       | Forged    | 0.51                     | 1.36 | 0.42 | 1.23 | 0.22 | 0.16 | "   |
| 3       | Forged    | 0.53                     | 1.30 | 0.36 | 1.19 | 0.31 | 0.03 | "   |
| 4       | Cast      | 0.56                     | 1.38 | 0.32 | 1.24 | 0.25 | 0.02 | "   |
| 5       | Cast      | 0.50                     | 1.32 | 0.35 | 1.19 | 0.24 | 0.21 | "   |
| 6       | Cast      | 0.51                     | 1.35 | 0.45 | 1.24 | 0.22 | 0.40 | "   |

The alloys find utility as a structural material in the fabrication of explosive warheads for use against both light and heavy military targets. For example, antipersonnel grenades, artillery and mortar shells, serial bombs as well as other explosive devices which utilize fragment pieces as a weapon can make use of the alloys of this invention.

Accordingly, the primary object of this invention is to provide an alloy steel that possesses desirable fragmentation characteristics when used in fabricating explosive warheads.

Another object of this invention is to provide a low alloy steel whose fragmentation characteristics are controlled by the inclusion of titanium as an alloying ingredient.

Heat treatment of the alloys in Table I were conducted in accordance with known hardening techniques so that large grained martensitic metallurgical structures with a titanium rich grain boundary network were produced.

Test results indicated that the higher the titanium content, the finer the fragmentation. These results are graphically shown in FIG. 1 and 2 of the drawings. From these results it can be seen that the addition of titanium to steels, which have been properly heat treated, produces a titanium-rich network that can be utilized to control fragmentation. Utilization of the techniques of this invention allows for the simple production of naturally fragmenting warheads. By selection of titanium content, warheads for use against both light and heavy targets can be obtained.

From an examination of the foregoing, it can be seen that the present invention provides a means for controlling the fragmentation characteristics of steel alloys in a simple and efficient manner. The invention provides steel alloys that are especially useful as structural materials in the fabrication of explosive warheads for use against military targets.

While the principle of this invention has been pointed out with particularity, it should be understood that various modifications and alterations can be made without departing from the spirit thereof, the scope of which is defined by the appended claims.

What is claimed is:

1. A fragmentation type steel alloy consisting of by weight about 0.02 to 0.4 percent titanium; about 0.50 to 0.60 percent carbon; about 1.30 to 1.40 percent manganese; about 1.15 to 1.25 percent chromium; about 0.30 to 0.50 percent silicon; about 0.20 to 0.30 vanadium; and the remainder substantially all iron.
2. An alloy in accordance with claim 1 containing about 0.02 percent titanium.
3. An alloy in accordance with claim 1 containing about 0.21 percent titanium.
4. An alloy in accordance with claim 1 containing about 0.40 percent titanium.

\* \* \* \* \*

15

20

25

30

35

40

45

50

55

60

65